

1

3,020,147

## PROCESS FOR THE HEAT HARDENING OF PELLETS COMPOSED OF ORES ON SINTER- ING GRATES

Karl-Heinz Boss, Bad Homburg vor der Höhe, Hans Rausch, Oberursel (Taunus), and Kurt Meyer, Frankfurt am Main, Germany, assignors to Metallgesellschaft Aktiengesellschaft, Frankfurt am Main, Germany

No Drawing. Filed Feb. 15, 1960, Ser. No. 8,483  
Claims priority, application Germany Mar. 25, 1959  
1 Claim. (Cl. 75—5)

This invention relates to the heat hardening of green pellets composed of iron ore and, in particular, is directed to the hardening of the pellets by means of hot gases.

It is known to convert fine-grained ores, particularly iron ores, into lumpy form by sintering them into cohesive cakes on a sintering band, if necessary, after previously crumbling and/or granulating the ores and to subsequently break up these cakes into pieces of suitable size. The heat required for carrying out this procedure can be supplied either by hot gases or solid fuel and also by a mixture of gas and solid fuel. It is likewise known to form fine-grained ores moistened with water into large spherical granular bodies with a diameter of 8 to 20 mm. in a granulating drum or on a granulating disc and then to hard-burn these bodies in a shaft furnace into non-cohesive pellets or balls with the aid of hot gases. It has also been proposed to apply this process to a moving grate or sintering band. In this case, the moist pellets, so-called green pellets, are charged onto the sintering band, after first preferably laying a protecting grate layer of finished burnt material on the band, then running the pellets under a gas dome where relatively warm gases are drawn through the bed of pellets to predry and preheat the pellets, then treating the bed with strong oxidizing gases under a second gas dome where the actual hard-burning is carried out, and finally cooling the bed in a third zone by cold air sucked through the charge. The pellets therefore travel successively through three horizontal zones with different gas atmospheres and at different temperatures arranged one following the other, as disclosed in the patent to Lellep, No. 2,750,272.

In this procedure, however, objections and difficulties are encountered which do not occur in the case of the conventional sintering of ore into cohesive sinter cakes.

As the raw relatively fragile green pellets are sensitive both to mechanical stressing and also to fluctuations in temperature, it is necessary to introduce various precautionary measures which have a detrimental effect both on the throughput capacity of the process as well as on the quality of the burnt product obtained. First, it is not possible to obtain as uniform and level a charge bed as in the case of the conventional sintering. Whereas in the conventional sintering process, the charge bed can be smoothed flat with a scraper arranged at a suitable height above the sintering band. This is not possible when burning green pellets, because the mechanically sensitive green pellets are seriously damaged and even to a great extent almost completely destroyed by the scraper. It has therefore hitherto been necessary to try to produce an absolutely level and uniform bed, which however results in that the lowermost portions of the bed are not heated to a sufficiently high temperature at the places where the pellets are piled up too high, whereas overheating of the grate cannot be avoided at the places where the pellets are not laid to a sufficient thickness. Furthermore, the thermal sensitivity of the green pellets requires very careful and consequently time-wasting drying and preheating treatment, before the actual burning process takes place, by

2

passing moderately warm gases at about 200 to 400° C. through the bed. The suction area of the grate to be made available for the first or preheating zone must therefore be in the same order of magnitude as the area of the actual burning zone in which gases at about 1100 to 1400° C. are drawn through the bed. It is understandable that, on this account, the total output of the sintering band expressed in tons of throughput per square meter of sintering surface and unit of time, for example a 24 hour day, is decreased considerably.

This invention enables both of the objections to the known burning process to be overcome simultaneously. This invention has discovered that a lowering of the gas suction pressure in the preheating zone to reduce the velocity of the flow of gas through the bed or pellets is sufficient in of itself to prevent the pellets from bursting even if the preheating in its previous sense were dispensed with and the green pellets treated initially and immediately with hot gases at about 1,000° C. and above. The invention has the advantages of simplicity and economy.

Thus the pellets are preheated for a short period of a few minutes with a gas having a temperature of about 1,000° C. or more which is practically identical with the pellet burning temperature. In drawing the gas through the bed of pellets at a lower speed in the preheating zone than in the hard burning zone, a pressure difference between the upper and lower surfaces of the bed amounting to about 20 to 60 mm. water of column (W.col.) is preferably used in the preheating zone and of 70 to 200 mm. W.col. in the hard burning zone.

Whereas, in the prior art processes for the hard burning of green pellets on a sintering band, the preheating zone constitutes a zone entirely separate from the actual burning zone in the direction of travel of the sintering band; the process of this invention enables the burning zone to overlap the drying zone to a considerable extent and consequently a better utilization is made of the expensive sintering grate surface area, with the result that a throughput of, for example, 19 to 21 metric tons per square meter of grate surface area in 24 hours are possible with a certain kind of ore, as compared with 10 to 11 tons per square meter in 24 hours for the same kind of ore without using the process of this invention.

In a further embodiment of this invention, an additional layer composed of perhardened or finished burnt pellets or graded pellet scrap is laid on top of the bed of green pellets on the sintering band. This layer can be spread without difficulty from a distributing bunker upon the bed of green pellets.

It has been found that this additional layer has sufficient mechanical strength to be smoothed by a scraper without the hard pellets or pellet scrap becoming damaged or destroyed. Moreover, the forces produced by the scraper are widely distributed so that the forces reaching the bed of raw green pellets are so small as to leave the green pellets practically undamaged.

By this means therefore, it is possible to form a bed on the sintering band which is just as uniform and smooth as in the case of conventional sintering.

The advantages of the method of this invention are shown by a comparison of the following specific examples. Example 1 is a test carried out according to the known state of the prior art. Example 2 shows that an increase in output cannot be attained by increasing the temperature of the gas during the green pellet drying period under process conditions unchanged from the prior art. Example 3 is the simplest form of carrying out the method of this invention. Example 4 is an improvement of the method of this invention which consists substantially in that, after shutting off the heating, still relatively hot gases, such as preheated air, are drawn through the bed with the result that the sensible heat of the upper and middle layers

is carried to the lowermost layer so that this heat content can be rendered available for hard-burning the pellets located in the lowermost layers. Examples 5 and 6 correspond with Examples 3 and 4 with the difference that an additional cover layer of preburnt pellets is spread upon the green pellets. This modification is recommended particularly when the green pellets consist of a material which is so sensitive that even when the gas vacuum is reduced according to this invention the green pellets do not withstand the direct contact with the hot gases at about 1000° C. without bursting. Instead of the additional layer being composed of preburnt pellets, pellet scrap, that is fragments of finished burnt pellets constituting more or less waste material, can be used in practice just as successfully.

The consumption figures concerning the quantities of heat used per kg. of pellets and obtained from the examples should only be considered as figures for comparing the examples with one another, because these represent values of the heat consumption without further recovery of waste heat, such as is customary in practical working. Therefore, all the comparison figures of the examples, that is of the examples carried out according to the prior art, as well as those representing the invention, are not inconsiderably less favorable than the values obtainable with the same methods in practical working.

#### EXAMPLE 1

##### *State of the prior art*

70 kg. of raw green pellets of magnetite containing about 64% Fe and 8% SiO<sub>2</sub> with a water content of about 9% and an average diameter of 15 to 20 mm. are spread to a depth of 33 cm. on a sinter grate having a surface area of 30 x 30 cm. after the metal grate has been first covered with a protective grate layer of burnt pellets to a depth of 10 cm. The total thickness of the layer is then 33+10=43 cm. A side layer of broken pellets with a grain size of 2 to 10 mm. is then poured between the green pellets and the side of the grate. In order to harden the green pellets by heat treatment, the grate is covered above the bed of green pellets with a hood in which a burner is located. The hardening of the pellets is carried out in the following stages:

(a) *Drying the green pellet.*—For a period of 15 minutes gases with a temperature of 300° C. are sucked through the charge at a vacuum of 80 to 100 mm. water column.

(b) *Heating up.*—During the next 13 minutes, the temperature of the gases sucked through the charge is increased from 300 to 1100° C. at a vacuum of 100 to 150 mm. water column.

(c) *Burning.*—For the burning operation, gases at a temperature of 1250° C. are sucked through the charge for 14 minutes until the pellets above the protective grate layer have reached this temperature. Then the charge is allowed to stand for 5 minutes without suction being applied.

(d) *Cooling.*—For 25 minutes, cooling air is forced through the grate from the bottom towards the top.

The pellets thus produced have an average strength of 300 to 400 kg. per pellet. The output of the sintering grate per square meter suction area and 24 hours is approximately 13 to 14 metric tons of finished pellets. During the different stages of the method, between 7 and 7.7 cubic meters of gas per minute were sucked through the charge. The heat consumption, calculated without beneficiation of the heat content of the finished product, was 1350 kcal./kg. burnt pellets.

#### EXAMPLE 2

With the same charge of green pellets on the sinter grate as in Example 1, the temperature of the drying gases at the same vacuum of 80 to 100 mm. water column is immediately increased to 1000° C. After a few minutes, the test had to be stopped. The reason for this was the premature

bursting of the green pellets in the upper layers which caused a reduction in the porosity of the bed charge and the stoppage of the passage of gas through the bed.

#### EXAMPLE 3

##### *The process of this invention*

The same green pellet bed charge as in Examples 1 and 2 was directly subjected from the beginning to hot gases at 1000° C., while the vacuum was maintained between 35 and 60 mm. water column during only the first 3 minutes and then increased to from 100 to 250 mm. water column. After 26 minutes, including the 3 minutes heating-up period, the heating was shut off because the temperature of the pellets above the grate protective layer had reached the temperature necessary for hardening. After allowing the charge to stand for 5 minutes without applying suction, the cooling with compressed air was started and, as in Example 1, lasted 25 minutes.

With this method, it was possible to reduce the total period of treatment by about 15 minutes and thereby attain an increase in output from 14 to 18 tons of finished product per square meter grate surface area. Although the pellets were of the same quality as in Example 1, the heat consumption per kg. of burnt pellets necessary for the burning was 700 kcal./kg. burnt pellets, i.e. less by about 50%. Also the thermal stress on the grate bars was less, as they reached a maximum temperature of 550° C.

#### EXAMPLE 4

As in Example 3, the green pellet bed charge was first treated with gases at 1000° C. The vacuum, which during the first 3 minutes was between 40 and 60 mm. water column, was then increased to 100 to 250 mm. water column, while the temperature of the hot gases was at the same time increased to 1250° C. After a burning period of 19 minutes, including the 3 minutes for heating up, the heating was shut off. The temperature above the protective grate layer had then reached 400 to 450° C.

While the hood remained over the charge, atmospheric air from above the burner hood was sucked through the bed charge. As a result, the air, being in contact with the still hot burner hood, became heated to about 400 to 500° C. The sucking in of preheated air was continued for a period of 9 minutes. Consequently, the sensible heat in the upper layers of the charge was carried into the lowermost layers and thus utilized for the hard-burning thereof.

As compared with Example 3, further improvements were attained, namely the output was now 20 tons per day per square meter grate area, the heat consumption up to the end of the heating period was 500 kcal./kg. burnt pellets, i.e., lower by about 25%, as compared with Example 1 it was 60 to 65% lower, the temperature in the grate bars reached only 340° C., and the quality of the burnt pellets was still good by having a strength of 250 to 350 kg. per pellet.

#### EXAMPLE 5

60 62 kg. of green pellets were charged to a height of 29 cm. onto the grate which was covered with a protective grate layer 10 cm. in thickness. Over this layer of green pellets, a layer of previously burned pellets ranging from 4 to 12 mm. in diameter was spread to a thickness of 4 cm. The bed charge was then treated in the same manner as in Example 3. As compared with Example 3, the charge of green pellets was more uniformly burnt. Particularly, the pellets directly below the covering layer were of better quality. The heat consumption was 770 kcal./kg. burnt pellets.

#### EXAMPLE 6

65 The sinter grate was charged in the manner as in Example 5. The same steps of burning were employed as in Example 4, that is, heating up with gases at about 1000° C. for 3 minutes, followed by burning with gases

at 1250° C. until about 400° C. was reached above the protective grate layer, then continuation of the suction until pellet hardening temperature was reached above the protective grate layer and then finally cooling with compressed air. The heat consumption was 595 kcal./kg. burnt pellets.

The operating data for the above examples is summarized in the following table for purpose of comparison.

as grate bars not heated above 600° C. will last for years. It is thus demonstrated that the process of this invention employing an initial high temperature drying and preheating of the raw green pellets while using a low volume of gas flow is a practical advance in the art.

Having now described the means by which the objects of the invention are obtained, we claim:

A process for hard-burning raw green pellets not greater

SINTER GRATE GREEN PELLET BED CHARGE

| Contents           | Ex. 1 | Ex. 2 | Ex. 3 | Ex. 4 | Ex. 5 | Ex. 6 |
|--------------------|-------|-------|-------|-------|-------|-------|
| Grate Layer:       |       |       |       |       |       |       |
| kgs.               | 20    | 20    | 20    | 20    | 20    | 20    |
| cms.               | 10    | 10    | 10    | 10    | 10    | 10    |
| Green Pellets:     |       |       |       |       |       |       |
| kgs.               | 70    | 70    | 70    | 70    | 62    | 62    |
| cms.               | 33    | 33    | 33    | 33    | 29    | 29    |
| Pellet Size, mmns. | 15-20 | 15-20 | 15-20 | 15-20 | 15-20 | 15-20 |
| Side Layer:        |       |       |       |       |       |       |
| kgs.               | 28    | 28    | 28    | 28    | 28    | 28    |
| cms.               | 2-3   | 2-3   | 2-3   | 2-3   | 2-3   | 2-3   |
| Pellet Size, mmns. | 2-10  | 2-10  | 2-10  | 2-10  | 2-10  | 2-10  |
| Cover Layer:       |       |       |       |       |       |       |
| kgs.               |       |       |       |       | 8     | 8     |
| cms.               |       |       |       |       | 4     | 4     |
| Pellet Size, mmns. |       |       |       |       | 15-20 | 15-20 |
| Total Charge, cms. | 43    | 43    | 43    | 43    | 43    | 43    |

DURATION OF THE INDIVIDUAL PERIODS

|                          |    |    |    |    |    |    |
|--------------------------|----|----|----|----|----|----|
| Drying, mins.            | 15 | 5  |    |    |    |    |
| Heating Up, mins.        | 13 | 3  | 3  | 3  | 3  | 3  |
| Burning, mins.           | 14 | 23 | 16 | 21 | 17 |    |
| Standing, mins.          | 5  | 5  |    | 5  |    |    |
| Continued Suction, mins. |    |    | 9  |    | 8  |    |
| Cooling, mins.           | 25 | 25 | 22 | 25 | 22 |    |
| Total Time, mins.        | 72 | 5  | 56 | 50 | 54 | 50 |

TEMPERATURES IN THE INDIVIDUAL PERIODS

|                        |           |       |           |       |           |       |
|------------------------|-----------|-------|-----------|-------|-----------|-------|
| Drying, °C.            | 300       | 1,000 |           |       |           |       |
| Heating Up, °C.        | 300-1,100 | 1,000 | 1,000     | 1,000 | 1,000     | 1,000 |
| Burning, °C.           | 1,250     | 1,250 | 1,250     | 1,250 | 1,250     | 1,250 |
| Standing, °C.          | 1,250     |       |           |       |           |       |
| Continued Suction, °C. |           |       | 1,000-500 |       | 1,000-500 |       |
| Cooling, °C.           | 20        | 20    | 20        | 20    | 20        | 20    |

QUANTITIES OF WASTE GAS CONSUMED IN THE INDIVIDUAL PERIODS

|                                                        |         |         |         |         |         |         |
|--------------------------------------------------------|---------|---------|---------|---------|---------|---------|
| Drying, Nm. <sup>3</sup> /min. <sup>1</sup>            | 7.7     | 7.7     |         |         |         |         |
| Heating Up, Nm. <sup>3</sup> /min. <sup>1</sup>        | 7.5     | 3.3     | 3.3     | 3.3     | 3.3     | 3.3     |
| Burning, Nm. <sup>3</sup> /min. <sup>1</sup>           | 7.5     | 4.2-4.0 | 4.2-4.0 | 4.2-4.0 | 4.2-4.0 | 4.2-4.0 |
| Standing, Nm. <sup>3</sup> /min. <sup>1</sup>          |         |         |         |         |         |         |
| Continued Suction, Nm. <sup>3</sup> /min. <sup>1</sup> |         |         | 3.8     | 3.8     | 3.8     |         |
| Cooling, Nm. <sup>3</sup> /min. <sup>1</sup>           | 7.5-7.0 | 5.5-6.0 | 5.5     | 5.5-6.0 | 5.5     |         |

VACUUM IN THE INDIVIDUAL PERIODS (OR PRESSURE DURING THE COOLING)

|                                                |         |         |         |         |         |         |
|------------------------------------------------|---------|---------|---------|---------|---------|---------|
| Drying, mmns/wat. col. <sup>2</sup>            | 80-100  | 200-300 |         |         |         |         |
| Heating Up, mmns/wat. col. <sup>2</sup>        | 90-130  | 40-60   | 40-60   | 40-60   | 40-60   | 40-60   |
| Burning, mmns/wat. col. <sup>2</sup>           | 140     | 100-250 | 100-250 | 100-250 | 100-250 | 100-250 |
| Standing, mmns/wat. col. <sup>2</sup>          |         | 0       |         |         |         |         |
| Continued Suction, mmns/wat. col. <sup>2</sup> | 100-200 | 180-200 | 200-90  | 200-90  | 180-200 | 200-90  |
| Cooling, mmns/wat. col. <sup>2</sup>           |         |         |         |         |         |         |

RESULTS

|                                                          |         |         |         |         |         |  |
|----------------------------------------------------------|---------|---------|---------|---------|---------|--|
| Output, Tons Per Day per sq. meter                       | 14.1    | 18.0    | 20.4    | 16.6    | 18.0    |  |
| Strength of Pellets, <sup>3</sup> kg. per pellet         | 300-400 | 300-350 | 250-350 | 300-400 | 300-350 |  |
| Grate Bar Temperature, °C.                               | 880     | 550     | 340     | 510     | 400     |  |
| Heat Consumption without recovery, Units per kg. pellets | 1,350   | 700     | 500     | 770     | 595     |  |

<sup>1</sup> Normal cubic meters per minute.

<sup>2</sup> Range of vacuums and pressure made to keep gas volume of flow substantially constant as porosity of bed changed during heating and cooling.

<sup>3</sup> Range of compression strengths of pellet samples taken from different parts of bed.

From the examples as detailed in the above table, it is seen that Examples 3 to 6 of this invention achieved at least a one-third increase in output over the prior art process of Example 1. Pellets were of acceptable strength, it being noted that pellets having a crushing strength of 100 kg. not to be shipped are acceptable, and pellets having a strength of 250 kg. are shipable. The grate bar temperatures are important as cast iron grate bars heated to above 732° C. have a life of but about two to three months in a sintering apparatus, where-

than about 20 mm. in diameter and having a moisture content of about 9% H<sub>2</sub>O and composed of fine-grained iron ore comprising forming a bed of pellets at rest upon a horizontally moving sinter grate, drawing hot gas at a temperature of from about 1000 to 1400° C. through said bed with a low velocity corresponding to a vacuum of from about 20-60 mm. water column to dry and preheat the pellets in the top of said bed to about the temperature of said hot gases without bursting the pellets and then increasing the vacuum to about 70-200 mm. water

column to increase the hot gas velocity to continue the heating of the pellets throughout the entire bed and thus burn and heat harden the unbroken pellets at a temperature of from about 1000 to 1400° C.

|           |               |               |
|-----------|---------------|---------------|
| 2,380,056 | Lloyd         | July 10, 1945 |
| 2,672,412 | Burrow et al. | Mar. 16, 1954 |
| 2,750,273 | Lellep        | June 12, 1956 |
| 2,789,895 | Nora          | Apr. 23, 1957 |

References Cited in the file of this patent

UNITED STATES PATENTS  
2,191,911 Greenawalt Feb. 27, 1940

|         |  |
|---------|--|
| 229,608 |  |
| 750,518 |  |
| 566,145 |  |

#### FOREIGN PATENTS

|               |               |
|---------------|---------------|
| Great Britain | Feb. 26, 1925 |
| Great Britain | June 20, 1956 |
| Canada        | Nov. 18, 1958 |